

## UNITED STATES PATENT OFFICE

TENNEY L. DAVIS, OF NORWELL, MASSACHUSETTS

## EXPLOSIVE AND SOLVENT THEREFOR

No Drawing.

Application filed November 8, 1927. Serial No. 231,981.

(GRANTED UNDER THE ACT OF MARCH 3, 1883, 22 STAT. L., 625)

The invention described herein may be used by the Government, or any of its officers or employees in prosecution of work for the Government, or by any other person in the United States, without payment to me of any royalty thereon, in accordance with the act of March 3, 1883.

The subject of this invention is an explosive and a solvent therefor.

10 The main object of this invention is the production of an explosive containing nitroguanidine and the provision of a solvent for such nitroguanidine.

15 Nitroguanidine is a well known explosive substance which is used both in high explosives and in propellant powders. As a high explosive it is about as powerful as trinitrotoluene and has been used in various mixtures with ammonium nitrate, paraffin, 20 etc., in bombs and for other purposes where an insensitive and powerful high explosive is needed. It has the further advantage of being exceptionally cool. The experiments of Vieille showed that this explosive produces a 25 temperature of only 907° C. Its coolness commends it for use in safety explosives. If incorporated into nitrocellulose powder it renders the powder flashless without impairing its ballistic power, and, as Vieille showed, 30 reduces erosion and lengthens the accuracy life of the gun.

At the present time, nitroguanidine is best prepared by treating guanidine nitrate with concentrated sulphuric acid. When the resulting solution or mixture is run into cold water the nitroguanidine precipitates out in the form of an impalpable white powder so finely divided that it may readily be incorporated into a nitrocellulose colloid which 40 may be shaped in the usual manner into smooth progressive burning powder grains.

The impalpable powder of nitroguanidine, prepared as described, is, however, not pure, for it contains a certain amount of the sulphuric acid from which it was precipitated. The nitroguanidine must be freed from this acid by recrystallization. Water appears to be the only feasible solvent, for hot water dissolves considerable nitroguanidine while 50 cold water dissolves but little. From the so-

lution, the nitroguanidine crystallizes out in splendid white needles of a fibrous texture which are difficult to powder and which are not proper to incorporate with colloided nitrocellulose. Nitro-guanidine is insoluble or sparingly soluble in the common organic solvents, such as alcohol, ether, acetic ester, carbon tetrachloride, chloroform, petroleum ether, naphtha, acetone, benzene, toluene, etc., etc., and none of these substances may be used for converting nitroguanidine alone or a mixture of nitrocellulose with nitroguanidine into a uniform colloid.

I have discovered that the aliphatic nitramine or nitro-amines as, for example, methyl nitro-amine, ethyl nitro-amine, dimethyl nitro-amine, methyl butyl nitro-amine, etc., are solvents for nitroguanidine. They convert the explosive into a non-crystalline mass and may be used for preparing colloids of nitroguanidine or of mixtures of nitrocellulose with nitro-guanidine. They have the advantage that they contain a nitro-group and so contribute to the vigor of the explosive. They have the further advantage that they are generally soluble both in water and in the usual organic solvents and thus permit the use of the usual solvents in the preparation of a nitro-cellulose nitro-guanidine colloid.

I claim:

1. An explosive comprising nitro-guanidine and an aliphatic nitro-amine.

2. A composition containing a nitro-cellulose nitro-guanidine explosive and an aliphatic nitroamine.

3. A composition containing a nitro-guanidine explosive and an aliphatic nitro-amine invigorator which is a solvent for the explosive.

4. A composition containing a nitro-guanidine explosive and an aliphatic nitro-amine invigorator.

5. The method of colloidizing nitro-guanidine consisting in treating the nitro-guanidine with a aliphatic nitro-amine.

TENNEY L. DAVIS.